

## UNITED STATES PATENT OFFICE

2,041,958

REFINING CELLULOSE FIBER FOR CON-  
VERSION INTO CELLULOSE DERIVA-  
TIVESGeorge A. Richter, Berlin, N. H., assignor to  
Brown Company, Berlin, N. H., a corporation  
of MaineNo Drawing. Application July 25, 1934,  
Serial No. 736,901

19 Claims. (Cl. 92—13)

This invention relates to the art of refining cellulose fiber or pulp more particularly for conversion into cellulose derivatives. While not limited thereto, it deals more specifically with a refining process designed to put preliberated cellulose fiber, such as sulphite or other chemical pulp, in such good condition for acetylation that cellulose acetate prepared therefrom is unsurpassed in quality by cellulose acetate prepared from high grade cotton or cotton linters, for instance, yielding cellulose acetate solutions substantially free of haze or turbidity, as hereinafter described.

In accordance with the present invention, preliberated cellulose fiber, such as sulphite or other chemical wood pulp, is put through the refining action of at least two different alkaline liquors. The first refining operation is accomplished with a comparatively dilute hot alkaline liquor, as such a liquor does well the work of ridding the pulp of the more easily removable non-alpha cellulose components, particularly when the pulp has undergone preliminary treatment with chlorine water, hypochlorite bleach liquor or other oxidizing or similar reagent that reacts upon residual ligneous matter present in the pulp. The second refining operation is accomplished with a strong caustic soda solution at sufficiently elevated temperature to avoid sensible mercerization of the pulp fibers, as I have found that a solution of such causticity as to have appreciable mercerizing activity at room or lower temperature does well the work of reducing markedly residual non-alpha cellulose components, especially pentosans, at non-mercerizing temperatures. It is most important that the pulp be refined or purified while being kept in a substantially unmercerized condition, since mercerized fiber does not respond properly to acetylation, particularly when it has been dried preparatory to acetylation and has thus undergone the marked shrinkage that attends the drying of mercerized fiber.

The refining operations practiced in accordance with my invention may advantageously be supplemented by other chemical treatments of the fiber. In addition to the preliminary treatment of the fiber already mentioned, the fiber is preferably bleached to whiteness after its initial refinement in the dilute, hot alkaline liquor. Indeed, the fiber may to advantage receive up to its secondary refinement the complete processing disclosed in Richter and Schur Patent No. 1,833,976 dated December 1, 1931, which processing includes the addition of soap or soap-form-

ing material, such as red oil, to the dilute, hot caustic soda solution serving as the pulp-refining reagent. As pointed out in that patent, the soap tends to emulsify or disperse certain undesirable residues present in the fiber and to promote the production of a refined fiber exceedingly low in its content of resinous, pitchy, gummy or other color-generating residues soluble in organic solvents. The initial refinement of the fiber may take place at a stock consistency of, say, 5% to 10 10%, in various other dilute, hot alkaline liquors whose alkalinity is equivalent to that of a caustic soda solution of, say, 0.5% to 2% strength. Thus, the hot alkaline liquor may be one containing calcium hydroxide, sodium carbonate, sodium 15 sulphide, or other suitable alkaline chemical.

Starting with ordinary unbleached sulphite wood pulp, which has an alpha cellulose content of about 87% and a pentosan content of about 5%, and putting it through the processing of the 20 aforementioned patent, one may arrive at a refined pulp having an alpha cellulose content of about 94.5% and a pentosan content of about 2.5%. Such refined pulp may undergo the secondary refinement or purification of the present 25 invention in bulk or sheet form. In either case, the pulp is brought into contact with excess caustic soda solution of at least about 10% to 14% strength and at sufficiently elevated temperature, say, 50° to 60° C., to avoid mercerization and its 30 undesirable effects on the pulp. The pulp may be maintained in contact with such solution for a period up to about one hour, at the end of which time the refining or purifying reaction has proceeded substantially to equilibrium. The fiber 35 is then washed preferably with water sufficiently hot to avoid mercerizing effects such as might result from the cooling of the refining liquor with cold water. The final product thus prepared has an alpha cellulose content of about 96% to 40 99% and a pentosan content of about 1% to 1.4%. It may be dried and subjected to acetylation as customarily to produce without difficulty excellent cellulose acetate, that is, cellulose acetate 45 that dissolves in the ordinary cellulose-acetate solvents to yield solutions of the desired freedom from color and haze and hence admirably adapted for use in making films, artificial silk, lacquers, etc. These results are attributable to the extremely low pentosan content and extraordi- 50 narily high alpha cellulose content of the refined wood pulp constituting the base of the cellulose acetate.

In carrying out the secondary refining operation on bulk pulp, the procedure may be to mix 55

the pulp with the strong alkaline liquor at a temperature of about 50° C. to produce a pulp suspension of, say, about 6% to 10% stock density. After a treating period of, say, about one hour, 5 the excess liquor may be removed from the stock by a thickener, centrifuge, or other suitable extractor, and thus be recovered for reuse in substantially undiluted condition. The stock may then be washed free of the remaining liquor with 10 hot water, as in a counter washer, with minimum dilution of the liquor. It is preferable to acidify the washed stock as with dilute sulphurous acid solution and to give it a final washing with water, thereby ensuring a complete removal of caustic soda. The washed stock may then be dried, 15 as by sheeting and drying on a pulp drier; or it may be otherwise dried and then shredded or fluffed for acetylation.

In carrying out the secondary refining operation of the present invention on sheeted pulp, 20 that is, pulp that has been sheeted and dried on a pulp drier to form thick sheets generally known as "drier sheets", the procedure may be to draw off the sheet progressively from a reel and feed 25 it through the strong alkaline liquor with a time of immersion of, say, 5 to 10 seconds, in the bath. The sheet as it leaves the bath is substantially uniformly saturated or soaked with solution. It is preferably lightly squeezed so as to remove 30 excess undiluted solution for reuse and is then reeled. The reeled sheet impregnated throughout with strong caustic soda solution is kept for, say, one hour, whereupon its caustic soda content is removed. The atmosphere in which the reeled 35 sheet is kept is preferably heated sufficiently so as to keep the solution in the sheet sufficiently hot to be without mercerizing effect on the fibers. If the sheet has previously been squeezed only lightly, it may be passed through press rolls on 40 its way to a washer, preferably of the counter current type, whereinto hot wash water is preferably delivered and wherein the caustic soda solution is recovered with minimum dilution. The press rolls may be set to reduce the solution 45 content of the sheet to not more than, say, about 50% to 60%, thereby leading to a recovery of more undiluted caustic soda solution for reuse. The washed sheet is preferably treated with dilute sulphurous acid solution, again washed, and 50 finally dried. The dried product is similar in its composition to that had from the treatment of bulk pulp. It may be shredded or fluffed for acetylation.

An alternative practice of treating sheeted pulp accordant with my invention may be generally similar to that followed in the viscose-making industry. Thus, a stack or succession of sheets may be immersed in strong, hot solution of caustic soda in the usual steeping press and the sheets may be permitted to soak therein for, say, thirty to sixty minutes, whereupon the plunger of the press may be applied to remove the excess or removable hot solution from the soaked sheets and the pressed sheets removed 60 from the press, suitably washed, and dried. Such a batch practice does away with the need of storing the sheets while they are impregnated with the caustic soda solution as hereinbefore described in connection with the processing of a continuous sheet.

I wish to emphasize the fact that for the purpose of the present invention, it is necessary to use a caustic soda solution of at least about 10% strength for effecting the secondary refining operation. The fact is that it is only when the

solution is of 12% to 14% or greater strength that the refined pulp may be acetylated with as good results as those realized from high grade cotton or cotton linters. As already indicated, this strong solution must be applied to, and removed from, the fiber at temperatures sufficient- 5 ly elevated to inhibit mercerizing effects, since otherwise the fiber would be impaired for acet- 10 ylation in the sense that it would become pas- sive toward the usual acetylating reagents. The secondary refining operation of the present in- 15 vention may, if desired, be applied to low grade cotton linters or to rag stocks that have been semi-purified and reduced to pulp, as such forms of cellulose can also be thus greatly improved 15 for acetylation.

While the principles of the present invention are applicable to various kinds of preliberated cellulose pulps, including kraft and soda wood pulps, they are of especial value when applied 20 to sulphite wood pulp, as such latter pulp is characterized by its comparatively low pentosan content as a result of the particular fiber-liber- 25 ating process used in its production, and, accord- 30 ingly, it can be processed in accordance with the present invention to produce a refined pulp of extremely low pentosan content more readily than such wood pulps as kraft and soda, which are of distinctly higher pentosan content to begin with. The fact is that when the conditions 35 of sulphite cooking or fiber-liberation are special- 40 ly chosen, the processing of the resulting sul- phite wood pulp in accordance with the present invention is attended by even better results than those hereinbefore indicated. Thus, if the bi- 45 sulphite cooking liquor is made up with a com- 50 bined SO<sub>2</sub> content of only about 1/2%, instead of the usual 1% or greater combined SO<sub>2</sub> content, and with a free SO<sub>2</sub> content of about 5% to 7%, and if cooking of the wood chips is per- 55 formed at somewhat lower temperatures than ordinarily, the processing of the resulting pulp as hereinbefore described leads to a refined prod- 60 uct whose pentosan content ranges from 0.5% to 1.0% and whose alpha cellulose content ranges 65 from 96% to 99%.

While refined cellulose fiber prepared by the process of the present invention is intended more especially for acetylation, nevertheless, it is ad- 70 mirably adapted for conversion into a wide va- 50 riety of cellulose derivatives, such as cellulose nit- 75 rate, cellulose xanthate, cuprammonium, cel- 80 lulose, cellulose ethers, etc., as its extremely low pentosan content and extraordinarily high alpha cellulose content bespeak cellulose derivatives and 85 end-products of highly desired physical and 90 chemical characteristics.

An important advantage of the process of the present invention is that it is an economical one in that the refinement of preliberated cellulose 95 fiber is first carried as far as is practicably pos- 60 sible in a comparatively inexpensive or dilute al- 65kaline liquor so that the more difficult subse- 70 quent or last-stage refinement can be performed in the more expensive or concentrated alkaline liquor with lower consumption of the alkali of such latter liquor, and, accordingly, with a greater number of uses of such liquor before it be- 75 comes so contaminated that it must be discarded or subjected to alkali-recovery operations.

I claim:

1. A process which comprises first refining preliberated cellulose pulp to higher alpha cel- 80 lulose content in an alkaline liquor of non-mer- 85 cerizing strength, and then refining the resulting 90

5 pulp to still higher alpha cellulose content in another liquor of mercerizing strength while maintaining such liquor sufficiently hot to avoid the mercerizing activity possessed thereby at room temperature.

6 2. A process which comprises first refining chemical wood pulp to higher alpha cellulose content in an alkaline liquor of non-mercerizing strength, then refining the resulting pulp to 10 still higher alpha cellulose content in another liquor of mercerizing strength while maintaining such liquor sufficiently hot to avoid the mercerizing activity possessed thereby at room temperature, and washing the pulp free of such liquor 15 while preserving the unmercerized condition of the pulp fibers.

20 3. A process which comprises refining cellulose pulp in a liquor of mercerizing strength and activity at room temperature but maintained sufficiently hot to avoid the mercerizing activity possessed thereby at room temperature, and washing the resulting pulp free of such liquor with wash water at sufficiently elevated temperature to preserve the unmercerized condition of 25 the pulp fibers.

25 4. A process which comprises refining cellulose pulp in a caustic soda solution of at least 10% strength while maintaining such solution at a temperature of at least about 50° C., and 30 washing the resulting pulp free of such liquor with sufficiently heated wash water to preserve the unmercerized condition of the pulp fibers.

35 5. A process which comprises subjecting cellulose fiber containing less than 10% of non-alpha cellulose impurities to the action of a caustic soda solution of at least about 10% strength under non-mercerizing, elevated temperature conditions to raise the alpha cellulose content of such fiber to upwards of 96%, and washing the 40 fiber free of such solution with wash water at sufficiently elevated temperature to maintain such solution at non-mercerizing activity.

45 6. A process which comprises subjecting cellulose fiber containing less than 10% of non-alpha cellulose impurities to the action of a caustic soda solution of at least about 10% strength under non-mercerizing, elevated temperature conditions to raise the alpha cellulose content of such fiber to upwards of 96%, washing the fiber 50 free of such solution with wash water at sufficiently elevated temperature to maintain such solution at non-mercerizing activity, and acetylating the unmercerized purified fiber.

55 7. A process which comprises immersing a sheet of purified wood pulp having an alpha cellulose content upwards of 90% in a caustic soda solution of at least about 10% strength under non-mercerizing, elevated temperature conditions, keeping the solution absorbed thereby in contact therewith for at least about one hour under such non-mercerizing temperature conditions, and washing the sheet free of the solution with wash water at sufficiently elevated temperature to maintain the solution at non-mercerizing activity.

60 8. A process which comprises immersing a sheet of purified wood pulp having an alpha cellulose content upwards of 90% in a caustic soda solution of at least about 10% strength under non-mercerizing, elevated temperature conditions, 65 keeping the solution absorbed thereby in contact therewith for at least about one hour under such non-mercerizing temperature conditions, washing the sheet free of the solution with wash water at sufficiently elevated temperature to maintain the solution at non-mercerizing activity, and

acetylating the unmercerized purified pulp constituting such sheet.

9. Substantially unmercerized cellulose fiber substantially free from ingredients soluble in a caustic soda solution of at least 10% strength at 5 a temperature of at least 50° C., said fiber having an alpha cellulose content of about 96% to 99% and a pentosan content not exceeding 1.5%.

10. Substantially unmercerized wood pulp substantially free from ingredients soluble in a caustic soda solution of at least 10% strength at a temperature of at least 50° C., said wood pulp having an alpha cellulose content of about 96% to 99% and a pentosan content not exceeding 1.5%.

15 11. A process which comprises first refining preliberated cellulose pulp to higher alpha cellulose content in an alkaline liquor of non-mercerizing strength, then refining the resulting pulp to still higher alpha cellulose content in an excess of another liquor of mercerizing strength while maintaining such liquor sufficiently hot to avoid the mercerizing activity possessed thereby at room temperature, removing a portion of the hot liquor from the pulp, and washing the pulp free of remaining liquor while preserving the unmercerized 20 condition of the pulp fibers.

25 12. A process which comprises first refining chemical wood pulp to higher alpha cellulose content in an alkaline liquor of non-mercerizing strength, then refining the resulting pulp to still 30 higher alpha cellulose content in an excess of another liquor whose alkalinity corresponds to a caustic soda solution of at least about 10% strength while maintaining such liquor sufficiently hot to avoid the mercerizing activity pos- 35 sessed thereby at room temperature, removing a portion of the hot liquor from the pulp, and washing the pulp free of remaining liquor while preserving the unmercerized condition of the pulp fibers.

40 13. A process which comprises refining preliberated cellulose pulp as a pulp suspension in an alkaline liquor of mercerizing strength and activity at room temperature but maintained sufficiently hot to avoid the mercerizing activity pos- 45 sessed thereby at room temperature, removing a portion of the hot liquor from the pulp, and washing the remaining liquor from the pulp with wash water at sufficiently elevated temperature to preserve the unmercerized condition of the pulp 50 fibers.

45 14. A process which comprises refining chemical wood pulp as a pulp suspension in an alkaline liquor whose alkalinity corresponds to a caustic soda solution of at least about 10% strength 55 while maintaining such liquor sufficiently hot to avoid the mercerizing activity possessed thereby at room temperature, removing a portion of such hot liquor from the pulp, and washing the remaining liquor from the pulp with wash water at 60 sufficiently elevated temperature to preserve the unmercerized condition of the pulp fibers.

55 15. A process which comprises refining preliberated cellulose pulp in sheet form in an alkaline soaking liquor of mercerizing strength and 65 activity at room temperature but maintained sufficiently hot to avoid the mercerizing activity possessed thereby at room temperature, squeezing a portion of the hot liquor from the soaked pulp 70 sheet, and washing the sheet free of the remaining liquor with wash water at sufficiently elevated temperature to maintain such liquor at non-mercerizing activity.

75 16. A process which comprises refining chemi-

cal wood pulp in sheet form in an alkaline soaking liquor whose alkalinity corresponds to a caustic soda solution of at least about 10% strength while maintaining such liquor sufficiently hot to avoid the mercerizing activity possessed thereby at room temperature, squeezing a portion of the hot liquor from the soaked pulp sheet, and washing the sheet free of the remaining liquor with wash water at sufficiently elevated temperature to maintain such liquor at non-mercerizing activity.

17. Substantially unmercerized, preliberated and refined cellulose fiber, said fiber having an alpha cellulose content of about 96% to 99%, a pentosan content not exceeding 1.5%, and capable

of undergoing conversion into a cellulose acetate solution substantially free of haze or turbidity.

18. A drier sheet of substantially unmercerized, refined cellulose fiber having an alpha cellulose content of about 96% to 99%, a pentosan content 5 not exceeding 1.5%, and capable of undergoing conversion into a cellulose acetate solution substantially free of haze or turbidity.

19. A drier sheet of substantially unmercerized, refined wood pulp having an alpha cellulose content of about 96% to 99%, a pentosan content not exceeding 1.5%, and capable of undergoing conversion into a cellulose acetate solution substantially free of haze or turbidity.

GEORGE A. RICHTER. 15